

## UNITED STATES PATENT OFFICE

1,981,396

PREPARATION OF CELLULOSE NITRO-  
ACETATE WITH NITRO-CELLULOSE

Cyril J. Staud, Rochester, N. Y., and Charles E. Waring, Dayton, Ohio, assignors to Eastman Kodak Company, Rochester, N. Y., a corporation of New York

No Drawing. Application December 31, 1930,  
Serial No. 505,958

6 Claims. (Cl. 260—101)

This invention relates to a process of forming cellulose-nitro-acetate by acetylating cellulose in the presence of nitro-cellulose which acts as a nitrating agent, in the presence of a solvent for nitro-cellulose, containing chloracetic acid, acetone, or the like.

An object of our invention is the preparation of a nitro-acetate derivative of cellulose by the use of cellulose nitrate as a nitrating agent. Although cellulose nitro-acetates have been prepared through the use of a variety of processes and nitration media, at no point has the use of cellulose nitrate as the nitrating agent been contemplated. No previous process has included the novel idea of exchanging some of the nitrate radicals of nitrocellulose for acetyl groups and simultaneously using these nitrate groups to nitrate the cellulose present in the reaction mixture. By the use of cellulose nitrate as the nitrating agent it makes possible a variation of proportions in predetermined quantities so that the nitro-acetate produced will be that desired by the operator. The conditions under which the cellulose nitrate might be used involved a considerable problem and required a rather extended experimental study to evolve conditions under which this reaction could be brought about. Addition of cellulose nitrate per se together with cellulose at the beginning of the acetylation process did not give as satisfactory results as might be desired, the resultant dope being full of black sludge and is subject to gel formation. The same phenomenon occurs when the cellulose nitrate in the dry form is added later in the acetylation or at any subsequent point during the preparation of cellulose acetate. In attempts to obviate this difficulty, the cellulose nitrate was added dissolved in acetic acid, but this proved unsatisfactory due to the formation of irreversible gels when the cellulose nitrate was added at the close of the acetylation. It was found by us that the solvents tried were unsuitable for the process due to the low water tolerance of the cellulose nitrate. Consequently the investigation was directed toward the trial of other solvents which were more energetic in their solvent action on the cellulose nitrate and solutions of which were capable of existing in the presence of a few per cent. of water. Among such solvents acetone and chloracetic acid were tried, both of which have proved satisfactory for this purpose, the chloracetic acid probably being the more satisfactory of the two, since the color of the final dope is better. It has also been found desirable to have acetic acid

present mixed with the solvent, this mixture being used to dissolve the cellulose nitrate.

In practice the solvent may be added to the acetic acid solution of the cellulose nitrate, or the cellulose nitrate may be added, dissolved in chloracetic acid, or acetone solution, the acetic anhydride being thereafter added.

Another object of the invention is to prepare a cellulose derivative, specifically a nitro-acetate which is soluble in acetone even when not subjected to hydrolysis subsequent to the acetylation. The product formed in Example III, given below, is soluble in acetone following acetylation, although a very short hydrolysis subsequent to the acetylation gives the product a better acetone solubility. This process involves the addition of fuming nitric acid as an aid to the nitration of the cotton linters by the cellulose nitrate and in this manner additional nitration will take place. Examples I and II do not contemplate the addition of the fuming nitric acid. For instance, if the operator wishes a product of low nitrogen content, fuming nitric acid is not added, but on the other hand, if a nitro-acetate of a higher nitrogen content is desired, the procedure in Example III is followed in which a higher nitrogen content is found in the resulting product than would be obtained by exchange of nitrate and acetate radicals.

The specific examples which follow illustrate the application of our invention to the formation of cellulose nitrate-acetates by the nitration of cellulose, with cellulose nitrate as the nitrating agent.

## Example I

About five pounds of a dope composed of cellulose nitrate containing approximately 12% nitrogen in solution in acetic acid in the ratio of 1 part of nitrocellulose to 12 parts of acetic acid, was dissolved in a mixture of about 17 to 20 pounds of acetic acid, about 5 pounds chloracetic acid, and about 45 cc. of a catalyst consisting of sulphuric and phosphoric acid in the proportion of 1:3. To this solution is added from 2 to 5 pounds of cotton linters. The whole is allowed to stand at room temperature for about 15 hours (20-25° C.). At the end of this time it was placed in a mixer and about 7-10 pounds of acetic anhydride (85%) were added. The outside temperature was maintained from 50 to 80° F. for about two hours, about 80 to 100° F. for approximately 5 hours, and about 100 to 130° F. for about sixteen hours, when a clear dope was obtained free from grain and fiber. The outside tempera-

ture was then lowered to about 100° F. and a hydrolysis mixture composed of 48 cc. concentrated hydrochloric acid, 1½ pounds of water and 5 pounds chloracetic acid was added with 5 thorough mixing. Hydrolysis was continued for 20 to 50 hours with temperature maintained at about 100° C. or until a sample showed that the cellulose ester was completely soluble in acetone. If desired, the material may be then precipitated, 10 washed and dried. The product was found to be soluble in acetone, chloroform, ethylene dichloride, ethyl acetate and 1.4-dioxan and to contain .69% nitrogen.

*Example II*

15 About ½ pound of cellulose nitrate containing approximately 12% nitrogen is dissolved in about 800 grams of acetone and is then thoroughly mixed with from 15 to 20 pounds of acetic acid and from 40-50 cc. of a mixed catalyst composed of sulphuric and phosphoric acids in the proportion of 1:3; from 2-5 pounds of cellulose linters are then added and the whole mass is allowed to stand at room temperature for from 15 to 20 hours. The material is then placed in a mixer and cooled to approximately 60° F. and from 5 to 10 pounds of 85% acetic anhydride are added. The temperature of about 60° F. is maintained from 1 to 3 hours and was then raised to about 80° F. and held at that point. This temperature is maintained for about 7 to 12 hours, or until a dope free from grain results. About 1500 to 2000 c. c. of a mixture of acetone and water in the ratio of 9:1 was added to hydrolyze the excess anhydride. A hydrolysis mixture composed of about 600 c. c. of water and about 3 liters of molten chloracetic acid is then added and the material is hydrolyzed for from 50 to 75 hours at about 120° F. or until a test sample showed the product to be soluble in acetone. The material may then be precipitated, washed and dried in the usual manner. The product is soluble in acetone, ethyl acetate, chloroform, chloroform-alcohol, 1:4 dioxan, and ethyl oxalate, and contains 1.04% nitrogen.

*Example III*

50 About 5 pounds of a solution of cellulose nitrate in acetic acid, having approximately 12 parts of acetic acid to 1 of cellulose nitrate, was mixed with about 13 pounds acetic acid, about 5 pounds chloracetic acid, and about 45 c. c. mixed catalyst (phosphoric and sulphuric acids in the proportion of 1 to 3), until a homogeneous dope was obtained. From 2 to 5 pounds cotton linters were then suspended in this dope and allowed to stand at room temperature for from 15 to 20 hours. The material was then transferred to a mixing apparatus and from 5 to 10 pounds 85% acetic anhydride was added. The temperature was kept at about 60° C. When the mass became pasty a solution of about 200 c. c. fuming nitric acid in about 500 c. c. of acetic acid was slowly added. A very grainy dope resulted. The temperature was slowly raised to about 30 to 50° C. and maintained at this temperature for 15 to 22 hours. The product at this point is soluble in acetone. However, it is preferred to subject the mixture to hydrolysis and a hydrolysis mixture of about the following proportions was added: 48 c. c. hydrochloric acid, 5 pounds chloracetic acid and ½ pound of water.

The hydrolysis was continued for from 25 to 40 hours at about 38° C. or until a nicely acetone-soluble product was procured. The material was then precipitated, washed, and dried in the usual manner. Analysis of this product showed 3.57% nitrogen.

80 Broadly our invention consists in the addition of cellulose to cellulose nitrate in a solvent which will make possible the nitration of the cellulose by the cellulose nitrate and then by use of acetic anhydride a cellulose nitroacetate is formed. One of the features of this invention is that some of the nitrate radicals are transferred from the cellulose nitrate to the cellulose and then upon acetylation the remaining available hydroxyl groups of the de-nitrated cellulose and those of the freshly nitrated cellulose are taken up by acetyl groups. It is understood that other known acetylation catalysts may be used than the one shown and that it is within the scope of this invention to apply this novel procedure to any acetylation reaction the only condition being that considerable solvent be present, together with the cellulose nitrate.

85 90 95 100 Any solvent may be used in this process which answers the requirements given previously, namely, a good solvent of nitrocellulose and its nitrocellulose solutions which must be capable of existing in a few per cent of water. Some further examples of this type of solvent are dichloroacetic acid, ethoxy acetic acid or methoxy acetic acid, or methyl ethyl ketone.

105 What we claim as our invention and desire to secure by Letters Patent of the United States is:

110 1. A process of making cellulose nitro-acetate which comprises introducing cellulose into a solution comprising cellulose nitrate and chloracetic acid and acetylating the resulting cellulosic mixture.

115 2. A process of making cellulose nitro-acetate which comprises introducing cellulose into a solution comprising cellulose nitrate and acetone and acetylating the resulting cellulosic mixture.

120 3. A process of making cellulose nitro-acetate which comprises introducing cellulose into cellulose nitrate in a solvent selected from the group consisting of the chlor-substituted acetic acids, the alkoxy substituted acetic acids and acetone and then acetylating the resulting mixture.

125 4. A process of making cellulose nitro-acetate which comprises introducing cellulose into cellulose nitrate in a solvent selected from the group consisting of the chlor-substituted acetic acids, the alkoxy substituted acetic acids and acetone, acetylating the resulting mixture and then treating the cellulose derivative formed with fuming nitric acid.

130 5. A process of making cellulose nitro-acetate which comprises introducing cellulose into a solution comprising cellulose nitrate and ethoxy acetic acid and acetylating the resulting cellulosic mixture.

135 6. A process of making cellulose nitro-acetate which comprises introducing cellulose into a solution comprising cellulose nitrate and acetone, acetylating the resulting cellulosic mixture, and treating the cellulose derivative formed with fuming nitric acid.

CYRIL J. STAUD.

CHARLES E. WARING. 145